

# UNITED STATES PATENT OFFICE.

BENNO STRAUSS, OF BREDENEY, GERMANY, ASSIGNOR, BY MESNE ASSIGNMENTS, TO THE CHEMICAL FOUNDATION, INC., A CORPORATION OF DELAWARE.

## ARTICLES WHICH REQUIRE HIGH RESISTANCE AGAINST CORROSION.

1,316,817.

Specification of Letters Patent. Patented Sept. 23, 1919.

No Drawing. Original application filed June 25, 1913, Serial No. 775,765. Divided and this application filed June 19, 1914, Serial No. 846,168. Renewed February 1, 1919. Serial No. 274,582.

*To all whom it may concern:*

Be it known that I, Professor Doctor BENNO STRAUSS, a citizen of the German Empire, residing at Bredeney, Germany, have invented certain new and useful Improvements in Articles Which Require High Resistance Against Corrosion, of which the following is a specification.

This application is a division of my application filed June 2, 1913, Serial No. 775,765.

This invention relates to articles such as gun barrels, turbine buckets and the like, which require a high resistance against corrosion, and it consists in the use of steel alloys for producing such articles, which contain from 6% to 25% chromium and from 20% to  $\frac{1}{2}\%$  nickel and not over 1% carbon.

20 In the production of such articles it has up to now been recommended to use nickel steel containing about 10% nickel or from 25% to 30% nickel.

It has now been proved by experiments 25 that alloys of the above named composition possess considerably higher power of resistance to corrosion than the previously used nickel steel alloys.

The great power of resistance of these 30 alloys will be evident from the following.

A bar from an alloy of 20% chromium and 2% nickel shows entirely shiny surfaces after it has been exposed for months to the influence of damp air, while bars of 35 ordinary steel and bars of nickel steel containing 10% nickel show considerably corroded surfaces when exposed to damp air for the same length of time, and even nickel steel with 25% nickel show corroded 40 surfaces.

Taking the loss in weight of mild steel as 100, a corroding test in sea water gave the following losses in weight for:

|                                       |    |
|---------------------------------------|----|
| 45 Nickel steel with 10% nickel       | 66 |
| Nickel steel with 25% nickel          | 44 |
| Steel with 10% chromium and 3% nickel | 16 |
| Steel with 20% chromium and 2% nickel | 9  |

At the same time the described alloy 50 nickel-chrom-steel possesses better qualities of strength than nickel steel containing 25% nickel, which has hitherto generally been considered as mostly rust proof.

The above steel alloys may be divided into

two groups namely, alloys which possess a 55 hardness over 380 (in accordance with Brinell) in the forged state; and such alloys which possess a hardness below 350 (also in accordance with Brinell) in the forged state.

To the first group belong alloys containing 60 6% chromium and 12% to 4% nickel or 12% chromium and 7% to  $\frac{1}{2}\%$  nickel or 18% chromium and 4% to  $\frac{1}{2}\%$  nickel.

Alloys of the first group which are difficult or almost impossible to work in the forged state can be made soft and easy to work if they are heated to a temperature between 500° C. and the critical point, and thereupon cooled quickly or slowly. The 70 critical point is situated in accordance with the composition of the alloy, between 720° C. and 780° C.

If this heating treatment be preceded by a heating up to 800° C. to 1000° C. with a 75 subsequent quick or slow cooling, the alloys will obtain in addition a great strength and toughness. By small additions of tungsten or vanadium the quality of strength of the alloys may be still more improved.

By means of a subsequent heating to 80 800° C. to 900° C. and subsequent quick or slow cooling, the alloys will again become hard and be difficult or impossible to work. This heating treatment forms consequently a means for hardening after working of articles produced from these alloys. These alloys may therefore be employed for the production of ball bearings as well as for the production of the balls therefor, 85 or generally speaking, to articles; which are exposed to rust or to the action of sea water.

The alloys belonging to the second group 90 may contain, for instance, the following proportions of chromium and nickel:

8% chromium and 20% to 10% nickel or 95 15% chromium and 20% to 5% nickel or 20% chromium to 25% chromium and 20% to 4% nickel.

Some alloys coming withing this group 100 are slightly magnetic and others non-magnetic, but all will obtain a very great toughness through heating up to 1100° C. to 1200° C. with subsequent quick cooling, and the slightly magnetic alloys will thereupon become unmagnetic.

I claim:

1. Articles which require a high resist-

ance against corrosion said articles being made from a steel alloy containing 6% to 25% chromium, 20% to  $\frac{1}{2}\%$  nickel and not over 1% carbon, the proportion of chromium increasing as the proportion of nickel decreases and vice versa.

5 2. Articles with a high resistance against corrosion which require to be unmagnetic, said articles being made from a steel alloy 10 containing 8% to 25% chromium, 20% to

$\frac{1}{2}\%$  nickel and not over 1% carbon, the proportion of chromium increasing as the proportion of nickel decreases and vice versa.

In testimony whereof the foregoing specification is signed in the presence of two 15 witnesses.

BLINNO STRAUSS. [L.S.]  
Witnesses:

ALBERT NUFER,  
FRANCES NUFER.